

Oct. 19, 1937.

P. M. CLARK

2,096,448

INSULATED ELECTRIC CABLE

Filed Jan. 6, 1934



Fig. 1



Fig. 2

Percy Morgan Clark INVENTOR.

BY Frank C. Hilberg

ATTORNEY.

## UNITED STATES PATENT OFFICE

2,096,448

## INSULATED ELECTRIC CABLE

Percy Morgan Clark, Parlin, N. J., assignor to  
 E. I. du Pont de Nemours & Company, Wil-  
 mington, Del., a corporation of Delaware

Application January 6, 1934, Serial No. 705,565

8 Claims. (Cl. 173—264)

This invention relates to an improved insulated electric cable, wherein a cellulose derivative composition is utilized as the surface coating, and is a continuation in part of my copending application 5 Serial No. 518,891, filed February 27, 1931.

Electric cables have previously been coated with cellulose derivative compositions thereby providing a finish on the cable which is tough, durable and flexible over a long period of time and which 10 is highly resistant to various deleterious agents. These compositions employ a considerable proportion of softener to give a film of the required toughness and flexibility to withstand the rough usage to which cables are subjected. A serious 15 objection to the use of these compositions is that the coatings produce a film having a considerable degree of tackiness and thermoplasticity largely due to the relatively high proportion of softener used. This objection has heretofore been partially overcome by baking or force drying the 20 coated cable before it is reeled for a prolonged storage period, but this procedure is unsatisfactory as it slows up production, adds to the expense of coating, and does not eliminate the characteristic 25 thermoplasticity of these coatings.

This invention has as an object, the provision of an improved insulated electric cable finished with a coating which is non-tacky and quick drying and which does not require prolonged force 30 drying or cause appreciable delay in reeling the cable subsequent to the coating step. A further object is to provide a cable finished with a coating which, although basically thermoplastic, is protected from tackiness and sticking during 35 prolonged storage. A still further object is the provision of a cable carrying a finish coat which is tough, durable, flexible and insulating.

These objects are accomplished by the following 40 invention wherein an insulated electric cable is coated with a cellulose derivative composition which contains a relatively incompatible non-volatile paraffin wax free mineral oil, a solvent softener incompatible with the mineral oil, the oil being present in an amount sufficient to be 45 exuded or spewed out as a thin top film, whereby the tackiness and thermoplasticity which otherwise would be present due to the softener is overcome.

In the drawing, Figure 1 is a diagrammatic 50 section of a cable produced according to the pres-

ent invention. Figure 2 is also a diagrammatic section of a cable prepared according to the present invention. In both figures, 1 represents an electrical conductor, 2 is a rubber or other insulating coating, 3 indicates a fabric layer over the 5 said insulating coating, and 4 represents a film of lacquer prepared according to the present invention having a very thin surface film of exuded mineral oil. The drawing is diagrammatic and the difference is not intended to be drawn to scale. 10

The composition of the present cable coating comprises a cellulose derivative such as cellulose nitrate, acetate or ether, a solvent softener in sufficient amount to give a film of the desired flexibility, a non-volatile mineral oil or other non-volatile oil incompatible with the cellulose derivative in sufficient amount to be exuded or spewed out and form a thin top film of oil when the coating dries. The usual lacquer solvents are used in sufficient quantity to give the composition 15 the desired viscosity, the composition being adapted for use either as a plastic or liquid coating.

By the term "solvent softener" as used herein and in the appended claims is meant those softeners which have an active solvent action on the cellulose derivative constituent of the composition as distinguished from those softeners generally classified as "non-solvent softeners" and which do not have an active solvent action on the 30 cellulose derivative, although possibly having some solvent action in the presence of alcohol or other solvents used in some coating compositions.

It is preferable also to use those solvent softeners which are highly incompatible with mineral 35 oil, because it is important to obtain the exudation or spewing out of the mineral oil with the use of as little of this oil as possible, the mineral oil if retained in sufficient quantity in the dried film having a tendency to weaken the film. Tricresyl 40 phosphate, a solvent softener is especially suited for this purpose, due to its extreme incompatibility with mineral oil. Triacetin and benzyl ether are also very incompatible with mineral oil and are also well suited for this purpose. However, other solvent softeners such as dibutyl tartrate, diethyl phthalate, dibutyl phthalate, et cetera, can be used satisfactorily.

The proportion of incompatible oil required to obtain proper exudation will depend upon the 50

type of cellulose derivative used and upon the particular softener used. Cellulose nitrate is the preferred cellulose derivative and it has been found that 10 parts by weight of cellulose nitrate with 5-15 parts by weight of softener require between 0.2 to 0.7 part by weight of mineral oil. It is not desirable to add mineral oil materially above 7% by weight of the cellulose nitrate. It has been found that if this ingredient is added materially above 7% by weight of the cellulose nitrate, for example about 10%, an abnormal and undesirable amount of exudation will frequently result. This causes a decidedly greasy film which adversely affects the process of coating the cable and the ultimate finish is likewise not acceptable. When this condition exists the adhesion of the coats applied subsequent to the first is very poor and in some cases in attempting to use such a composition under standard methods of coating is entirely inoperative. When the exudation is excessive the wiper (usually a rubber nipple surrounding the cable during coating operations) simply wipes off the freshly applied coating because the oily surface of the first coating precludes any degree of adhesion for subsequently applied coats. Further, this oiliness is frequently of such magnitude as to present an unsightly appearance and will transfer the oil to anyone handling the cable or to objects or covers coming in contact with it. The rapid accumulation of dust on the oily surface during storage and in use likewise presents additional adverse factors.

Cellulose acetate is much more incompatible with mineral oil than cellulose nitrate and from 0.1 to 0.5 part by weight of mineral oil to 10 parts of cellulose acetate form the preferred range. On the other hand, the cellulose ethers are more compatible with mineral oil than cellulose nitrate and 1.5 to 2.5 parts by weight of mineral oil must ordinarily be added to 10 parts of cellulose ether, even though a solvent softener highly incompatible with the mineral oil be used.

Due to the compatibility of cellulose ethers with mineral oil, it is not desirable to use solvent softeners having but slight incompatibility with mineral oil because the proportion of mineral oil that must be added to obtain exudation is so great as to give a materially weakened film. The solvent softener should be present however in sufficient amount to give the desired flexibility and the mineral oil in an amount just sufficient to exude as a thin top layer. It is not necessary that the oily top layer be so thick as to be clearly obvious to the eye, since a thin coat not perceptible to the eye, but sufficient to cause a cable coated with the composition to slip when pulled through the fingers, as contrasted to the sticking action of a cable coated with prior art high softener content lacquers, is sufficient to prevent coils of lacquered cable from sticking together even though stored at relatively high temperatures.

The non-volatile, relatively incompatible oil used in the composition as a coating for cables is preferably a highly purified, non-volatile paraffin free mineral oil of a viscous nature, such as "Nujol", "Primol", water white Russian oil, and high grade lubricating oils, all of which are non-volatile, oily paraffin or naphthene base hydrocarbons.

Resins may for the first time be used satisfactorily in these highly flexible coating compositions and are valuable in increasing the gloss, build, adhesion and insulating properties of the cable finish and also to decrease inflammability. The

use of thermoplastic resins in the finishes for the present purpose has heretofore been impractical, due to the stickiness of the film when exposed to elevated storage temperatures, but by the use of an incompatible non-volatile oil, this difficulty is overcome. Any of the resins used in cellulose derivative coating compositions are suitable for the present purpose, such as natural and treated natural resins and synthetic resins of the polyhydric alcohol-polybasic acid type, with or without modifiers such as drying oils, non-drying oils, etc., phenolaldehyde type, polymerized vinyl compounds, et cetera, provided that the finished composition has the properties necessary for a commercially practicable product for a coating composition.

As will be understood by those skilled in the art, the cellulose derivative, solvent softener, incompatible oil and, if desired, resin, are dissolved in suitable solvents, such as a mixture of ethyl acetate, ethyl alcohol and toluol, and the resulting solution, with or without coloring matter, fillers, et cetera, is applied to the surface of a cable and the solvent allowed to evaporate. If desired, the amount of solvent may be so reduced as to give a plastic composition instead of a lacquer or of a viscous composition.

The following examples are given to illustrate the compositions for the cables and not by way of limitation. The parts are by weight:

*Example 1.—Clear cable lacquer*

|                     |       |
|---------------------|-------|
| Nitrocellulose      | 12.5  |
| Tricresyl phosphate | 15.5  |
| "Nujol"             | 00.7  |
| Ethyl acetate       | 25.0  |
| Denatured alcohol   | 15.0  |
| Toluol              | 31.3  |
|                     | 100.0 |

*Example 2.—Black cable lacquer*

|                                  |       |
|----------------------------------|-------|
| Nitrocellulose                   | 12.5  |
| Tricresyl phosphate              | 15.5  |
| "Primol"                         | 00.7  |
| Ethyl acetate                    | 24.5  |
| Denatured alcohol                | 15.0  |
| Toluol                           | 31.3  |
| Nigrosine black (spirit soluble) | 00.5  |
|                                  | 100.0 |

*Example 3.—Cable lacquer (using a natural resin)*

|                         |       |
|-------------------------|-------|
| Nitrocellulose          | 13.0  |
| Tricresyl phosphate     | 9.0   |
| Damar resin             | 9.0   |
| Water white Russian oil | 0.7   |
| Ethyl acetate           | 22.0  |
| Toluol                  | 20.3  |
| Benzol                  | 16.0  |
| Denatured alcohol       | 10.0  |
|                         | 100.0 |

*Example 4.—Cable lacquer (using a synthetic resin)*

|                     |       |
|---------------------|-------|
| Nitrocellulose      | 15.0  |
| Tricresyl phosphate | 18.0  |
| Synthetic resin     | 10.0  |
| Ethyl acetate       | 25.0  |
| Benzol              | 24.3  |
| Denatured alcohol   | 7.0   |
| "Nujol"             | 0.7   |
|                     | 100.0 |

The synthetic resin used in this example is a reaction product of:

|                    | Per cent |
|--------------------|----------|
| Phthalic anhydride | 39.3     |
| 5 Glycerine        | 6.0      |
| Diethylene glycol  | 21.2     |
| Cocoanut oil       | 33.5     |
|                    | 100.0    |

10 The resin is prepared by heating the glycerine, diethylene glycol and cocoanut oil in a closed vessel fitted with a condenser for about 3 hours at 480° F. The mixture is cooled slightly and the phthalic anhydride added. The heating is then continued at 450° F. for 2-3 hours or until an acid number of 22 is reached.

Example 5.—Cable lacquer (cellulose acetate)

|                      |       |
|----------------------|-------|
| 20 Cellulose acetate | 12.0  |
| Triacetin            | 12.0  |
| Mineral oil          | 0.8   |
| Acetone              | 50.2  |
| Toluol               | 10.0  |
| 25 Denatured alcohol | 10.0  |
| Diacetone alcohol    | 5.0   |
|                      | 100.0 |

30 Example 6.—Cable lacquer (ethyl cellulose)

|                     |       |
|---------------------|-------|
| Ethyl cellulose     | 15.0  |
| Tricresyl phosphate | 15.0  |
| Mineral oil         | 0.8   |
| Toluol              | 2.5   |
| 35 Ethyl acetate    | 42.5  |
| Denatured alcohol   | 10.0  |
|                     | 100.0 |

40 Example 7.—Cable lacquer (benzyl cellulose)

|                     |       |
|---------------------|-------|
| Benzyl cellulose    | 12.0  |
| Tricresyl phosphate | 6.0   |
| Mineral oil         | 2.5   |
| 45 Ethyl acetate    | 15.0  |
| Toluol              | 54.5  |
| Denatured alcohol   | 10.0  |
|                     | 100.0 |

50 Example 8.—Cable plastic

|                     |       |
|---------------------|-------|
| Nitrocellulose      | 27.5  |
| Tricresyl phosphate | 37.2  |
| Denatured alcohol   | 7.1   |
| 55 Mineral oil      | 0.6   |
| Magnesium carbonate | 27.6  |
|                     | 100.0 |

60 These compositions are material improvements over those heretofore known, as the thin oily top layer eliminates the tackiness of the film in a much shorter period of drying and consequently prolonged baking and cooling of coated cables before reeling is not essential. It has been found that twice the speed in passage of the cable through the drying tower is permitted and also that the temperature in the drying tower may be reduced. It is possible to put many more 70 coats of lacquer on a cable than previously, without trouble being caused by tackiness of the film. Furthermore, cables coated with this composition may be reeled and stored at relatively high temperatures without sticking together or 75 marring the finish.

The thin oily film on the surface of the finish not only protects it in storage and handling, but adds appreciably to the appearance of the finish, giving a smooth, uniform surface.

The use of an incompatible, non-volatile oil 5 allows the proportion of softener in the composition to be increased without causing tackiness, thereby giving a more flexible finish, a feature particularly desirable in the cable coating art. Also resins may be used in the present compositions in substantial quantities, thereby giving a coating of increased gloss, build, adhesion and insulating properties, and reducing the inflammability of the finish. Heretofore the use of 10 resins has been impractical in compositions 15 designed for coating cable, because of their thermoplasticity.

The herein disclosed invention may be applied to practically any electrical cable. Particularly 20 good results have been obtained by coating a conventional cable having a conductor with layers of rubber and fabric with any of the compositions herein disclosed so that the exterior of the coated cable will have a layer of the cellulose derivative composition and exuded therefrom a 25 thin surface film of non-volatile mineral oil.

As many widely different embodiments of the 30 invention may be made without departing from the spirit and scope thereof, it is to be understood that I do not limit myself to the specific 35 embodiments thereof except as defined in the appended claims.

I claim:

1. A flexible electric cable coated with a tough, 35 durable insulating surface film comprising a cellulose derivative, solvent softener, and an incompatible non-volatile mineral oil, and having an exuded surface layer of non-volatile mineral oil over said surface film.

2. A flexible electric cable coated with a tough, 40 durable insulating surface film comprising cellulose derivative, solvent softener, a resin, and an incompatible non-volatile mineral oil, and having an exuded surface layer of non-volatile mineral oil over said film.

3. A flexible electric cable coated with a tough, 45 durable insulating surface film comprising cellulose nitrate, tricresyl phosphate, and an incompatible non-volatile mineral oil, and having a surface layer of non-volatile mineral oil over said film.

4. A flexible electric cable coated with a composition comprising 10 parts by weight of cellulose nitrate, 5-15 parts of tricresyl phosphate, 55 and 0.2 to 0.7 part of an incompatible non-volatile mineral oil, said composition when free from volatile solvents being tough, durable, insulating, and having a thin surface film of the said mineral oil.

5. A flexible electric cable coated with a tough, 60 durable insulating surface film comprising cellulose nitrate, tricresyl phosphate and from 0.02 to 0.07 part by weight of the cellulose nitrate of an incompatible non-volatile mineral oil and having a thin surface layer of non-volatile mineral oil of said film.

6. A flexible electric cable comprising a rubber 65 coated metallic conductor having a fabric coating over the rubber, said cable having a tough, durable insulating surface coating thereon of a composition comprising cellulose nitrate, tricresyl phosphate and from 0.02 to 0.07 part by weight of the cellulose nitrate of an incompatible non-volatile mineral oil and having a thin sur- 75

face layer of non-volatile mineral oil on said surface coating.

7. A flexible electric cable comprising a rubber coated metallic conductor having a fabric coating over the rubber, said cable having a tough, durable insulating surface coating thereon of a composition comprising 100 parts of cellulose nitrate, 50 to 150 parts by weight of tricresyl phosphate and 2 to 7 parts by weight of an incompatible non-volatile mineral oil and having a thin surface layer of non-volatile mineral oil on said surface coating.
- 10 8. An electric cable lacquer having substantial-

ly the same physical properties as the composition having the following formula:

|                     | Per cent |
|---------------------|----------|
| Nitrocellulose      | 12.5     |
| Tricresyl phosphate | 15.5     |
| Mineral oil         | 00.7     |
| Ethyl acetate       | 25.0     |
| Alcohol             | 15.0     |
| Toluol              | 31.3     |

said properties of the dried film including toughness, durability, high insulation, and said dried film having a thin exuded film of the mineral oil.

10 PERCY MORGAN CLARK